

# United States Patent

[19]

Pitchford et al.

[11] 3,919,072

[45] Nov. 11, 1975

[54] **RESINS FROM HIGH BOILING HYDROCARBONS AND ASPHALTS CONTAINING THE SAME**

[75] Inventors: **Armin C. Pitchford; Gene N. Woodruff**, both of Bartlesville, Okla.

[73] Assignee: **Phillips Petroleum Company**, Bartlesville, Okla.

[22] Filed: **Sept. 17, 1973**

[21] Appl. No.: **398,083**

[52] U.S. Cl. .... **208/4**; 208/6; 208/23; 208/39; 208/44; 208/45

[51] Int. Cl. .... **C07C 3/08**

[58] Field of Search ..... 208/4, 6, 23, 39, 44, 45

[56] **References Cited**

UNITED STATES PATENTS

|           |         |                 |        |
|-----------|---------|-----------------|--------|
| 2,179,988 | 11/1939 | Whitacre .....  | 208/4  |
| 2,627,498 | 2/1953  | Fink et al..... | 208/4  |
| 2,687,989 | 8/1954  | Goodwin.....    | 208/6  |
| 2,691,621 | 10/1954 | Gagle.....      | 208/23 |
| 2,773,004 | 12/1956 | Martin .....    | 208/45 |

|           |         |                    |        |
|-----------|---------|--------------------|--------|
| 2,774,724 | 12/1956 | Watson .....       | 208/6  |
| 2,904,494 | 9/1959  | Griffin .....      | 208/23 |
| 3,338,813 | 8/1967  | Van Pool .....     | 208/6  |
| 3,440,074 | 4/1969  | Stern, et al. .... | 208/23 |
| 3,462,359 | 8/1969  | Fauber.....        | 208/23 |
| 3,628,975 | 12/1971 | Van Pool .....     | 208/44 |

Primary Examiner—Veronica O'Keefe

[57] **ABSTRACT**

An aromatic oil say from catalytic cracking of hydrocarbon oil and/or a paraffinic oil as from solvent deasphalting of topped crude is air blown at elevated temperature and then further treated at elevated temperature in the presence of a catalyst, e.g., zinc chloride, to produce a hydrocarbon resin. The oil in which the resin has been produced is combined with a topped crude from which asphalt is to be produced or with an asphalt following which the admixture thus obtained is subjected to vacuum distillation or to a solvent deasphalting to remove unreacted or non-resinous, petroleum-derived fractions. An asphalt suitable for paving, having improved ductility and other properties, is obtained.

10 Claims, No Drawings

RESINS FROM HIGH BOILING HYDROCARBONS  
AND ASPHALTS CONTAINING THE SAME

This invention relates to the production of an improved asphalt composition. More particularly it relates to the production of an asphaltic resin containing asphalt composition and to the production of such a resin from an oil, e.g., a waxy crude oil, as distinguished from a petroleum residuum or asphalt. In one of its aspects, the invention can produce a final product containing in an asphalt, obtained upon vacuum reduction or a solvent extraction, a desired improved or increased amount or proportion of resinous material as distinguished from asphaltenes. In another of its aspects, the invention relates to the production of resinous materials from a petroleum oil, e.g., an oil derived from a synthetic crude oil obtained by catalytic cracking a virgin gas oil, a solvent gas oil, a heavy residual oil, a whole crude oil, and similar feedstocks.

The terms employed herein, e.g., "oil," "resin," "petroleum residuum," etc., have generally accepted meanings in the petroleum refining art and are employed to convey said meanings.

During the refining of certain crude oils an excess of a particular distillate or residual fraction may be produced while a shortage of another component will occur. Frequently this component can be of value in the preparation of a refined product for some specific application. Therefore, it is advantageous to convert a less desirable fraction of the crude oil to the most useful product without altering the overall crude charged to the refinery. Thus a change in refinery operation is made.

An example of this situation exists when a waxy crude oil is used to produce a distillate fuel and an asphaltic residue containing a deficiency of asphaltic resins. Asphaltic resins are necessary to impart certain characteristics to the asphalt and to overcome the adverse effects of the excess wax, which remains in the asphalt phase after vacuum flash distillation or solvent deasphalting of the oil, as with propane or with a mixed solvent, e.g., propane and butanes.

In one of its concepts, this invention provides a two stage process for preparing a resin-containing additive for improving the quality of asphalts, e.g., as derived from a waxy crude oil, which involves (1) air blowing of an aromatic oil or a heavy vacuum gas oil and (2) subsequently treating the airblown product with a catalyst, say, zinc chloride, at an elevated temperature such that there is formed in the oil a substantial proportion of resin.

In another of its concepts, the invention provides a process in which a resin-containing fraction or resin is added to an asphalt, or to a topped crude from which asphalt is to be prepared, to increase the resin content of the asphalt without substantially increasing the asphaltene content of the resulting blend, which comprises adding a resin or resin-containing fraction or petroleum resin to a topped crude and subjecting the admixture to a vacuum distillation thus to prepare a paving grade asphalt. In a further concept of the invention, the admixture is solvent deasphalting to obtain such a grade of asphalt. In the operation just described the resin remains in the asphalt to improve considerably its properties, e.g., ductility, etc.

It is known in the art to air-blow petroleum residuum at about 300°-500°F for, say, about 600 minutes and to

then subject the air-blown material, thus obtained, to a polymerization treatment as by heating it in the presence of aluminum chloride at 300°-400°F for 20 to 30 minutes.

We have conceived that an oil, as distinguished from a petroleum residuum, for example a bottoms obtained from a synthetic crude oil obtained by catalytically cracking a virgin gas oil or a solvent gas oil, as obtained from a topped crude by a propane-butane extraction, can be converted to a resin or resin-containing material or additive which then can be incorporated into a topped crude, as herein described, from which asphalt is to be prepared, and the admixture thus obtained processed to produce paving grade asphalt by a vacuum distillation or a solvent deasphalting to remove unreacted oil or gas oil therefrom, the product thus obtained being resin-enriched and possessing due to the presence therein of the added resin, considerably improved ductility and other properties.

An object of this invention is to prepare a petroleum resin. Another object of this invention is to prepare an improved asphalt derived from petroleum. A still further object of this invention is to prepare a resin to be incorporated into an asphalt, thus to obtain a product suitable for paving use, and other uses, without however increasing asphaltenes content. A still further object of the invention is to incorporate a petroleum resin, prepared according to the invention, into a topped crude from which an asphalt is to be prepared or into an asphalt. Another object of the invention is to produce an asphalt of improved properties from an oil low in resin content.

Other aspects, concepts, object and the several advantages of the invention are apparent from a study of this disclosure and the appended claims.

According to the present invention, an oil such as herein described is heated and air blown and still later while at an elevated temperature is further heated in presence of a catalyst which will produce resinous materials in the air-blown material, while avoiding the formation of asphaltenes, say,  $ZnCl_2$ ,  $FeCl_3$  and  $SnCl_4$ , as distinguished from  $CuCl_2$  and  $SnCl_4$ , to produce a resin or resin-containing material suitable for incorporation into a topped crude to be converted to asphalt, say, a paving grade quality. Also according to the present invention, a petroleum derived resin as herein described, as it may be contained in an oil in which produced, is incorporated into an oil to be converted to an asphalt which comprises admixing said material and said oil, e.g., topped crude or a solvent gas oil and then producing an asphalt in known manner, obtaining an asphalt of, say, paving quality, having properties considerably better than otherwise obtained to date in the art from such topped crudes and such solvent gas oils.

Generally, the resin-containing material will improve to an extent the properties of the final asphalt even when added in small proportions of the order of about five percent or even less. However, for now desirable in uses there will be incorporated into the topped crude or asphalt, or the like, from about 1 percent up to equal proportions or even more of the resin-containing material depending upon the natures of the materials to be admixed and further treated. Thus, one skilled in the art in possession of this disclosure having studied the same will understand that for each oil, treated according to the invention, and for each set of conditions of treatment, there will be a certain proportion of beneficial resin contained therein and therefore this will have

to be taken into account in admixing the treated oil containing the resin with the topped crude or asphalt to be benefited.

Thus according to the present invention, in one of its broad concepts, a petroleum fraction or oil is treated to produce a petroleum derived resin containing oil or oily material which is then admixed with a topped crude or asphalt, or equivalent material, from which by vacuum reduction or solvent extraction a final asphalt is obtained, as herein described.

The invention will now be described further with respect to the application of feedstocks, used for the preparation of the synthetic asphalt resins or resin-containing material, as given in Table I.

Table I  
PROPERTIES OF FEEDSTOCKS USED IN THE PREPARATION OF  
SYNTHETIC ASPHALT RESINS

|                             | Syn Tower Bottoms* |        |        | Solvent Gas Oil |
|-----------------------------|--------------------|--------|--------|-----------------|
| Identification              | A                  | B      | C      | D               |
| API Gravity at 60 F         | 6.8                | 13.6   | 3.8    | 23.2            |
| Specific Gravity, 60/60 F   | 1.0231             | 0.9752 | 1.0458 | 0.9147          |
| Viscosity, SFS, 122 F       | 27.0               | 47.6   | 52.2   | —               |
| Viscosity, SUS, 180 F       | —                  | —      | —      | 177.6           |
| Viscosity, SUS, 210 F       | —                  | —      | —      | 105.8           |
| Pentane Insolubles, Wt %    | 11.8               | 5.9    | —      | —               |
| Carbon Residue, Rams., Wt % | 7.86               | —      | —      | 0.78            |
| Elemental Analyses, Wt %    |                    |        |        |                 |
| Carbon                      | 89.2               | 88.47  |        |                 |
| Hydrogen                    | 8.7                | 11.25  |        |                 |
| Oxygen                      | 0.14               | —      |        |                 |
| Nitrogen                    | 0.09               | —      |        | 0.14            |
| Sulfur                      | 1.42               | —      | —      | 0.77            |
| Metals, ppm                 |                    |        |        |                 |
| Nickel                      | —                  | —      | —      | 0.7             |
| Vanadium                    | —                  | —      | —      | <0.3            |
| Iron                        | —                  | —      | —      | 2               |
| Distillation, ASTM D 1160   |                    |        |        |                 |
| IBP, °F                     | 577                | 564    | 564    | 780             |
| 2 %                         | 616                | 571    | 655    | 805             |
| 5 %                         | 703                | 680    | 724    | 853             |
| 10 %                        | 737                | 730    | 755    | 877             |
| 20 %                        | 776                | 768    | 789    | 913             |
| 30 %                        | 805                | 802    | 817    | 949             |
| 40 %                        | 822                | 819    | 841    | 972             |
| 50 %                        | 839                | 847    | 859    | 985             |
| Distillation Residue        |                    |        |        |                 |
| Per Cent of Feed            | 50                 | 50     | 50     | 61.8            |
| Viscosity, SFS, 210 F       | 13.1               | 7.5    | 31.4   | 18.4            |

\*Bottoms of a fractionator from the catalytic cracking unit.

To demonstrate the operability of the proposed process the sample of syntower bottoms designated as Sample A in the above tabulation was first air blown at conditions presented in Table II. Included in Table II

45 Table II shows properties of asphaltic resins derived from syn tower bottoms by air blowing and catalytic treatment in a second stage.

Table II  
PREPARATION AND PROPERTIES OF ASPHALTIC RESINS PREPARED FROM  
SYN TOWER BOTTOMS

| Feedstock                 | First Stage |                     | Second Stage      |                   | J                 |
|---------------------------|-------------|---------------------|-------------------|-------------------|-------------------|
|                           | Air Blowing | Catalytic Treatment | F                 | H                 | Blend*            |
| Run Number                | A           |                     | F                 | H                 |                   |
| Material Charged          |             |                     | F                 | H                 |                   |
| Catalyst Used             |             | none                | ZnCl <sub>2</sub> | ZnCl <sub>2</sub> | ZnCl <sub>2</sub> |
| Wt % Catalyst             |             | none                | 1.0               | 1.0               | —                 |
| Gas used in test          |             | Air                 | Nat.Gas           | Nat.Gas           | —                 |
| Gas Rate, SCFH            |             | 2.0                 | 1                 | 1                 | —                 |
| Temperature, F            |             | 492                 | 540               | 565               | —                 |
| Reaction Time, Hours      |             | 3.5                 | 6.0               | 7.0               | —                 |
| API Gravity at 60 F       | 13.6        | 8.3                 | 6.8               | 5.9               | 6.7               |
| Specific Gravity, 60/60 F | 0.9752      | 1.0122              | 1.0231            | 1.0298            | 1.0239            |
| ASTM D 1160 Distillation  |             |                     |                   |                   |                   |
| IBP, F                    | 564         | 705                 | 725               | —                 | 730               |
| 2%                        | 571         | 749                 | 755               | 768               | 768               |
| 5%                        | 680         | 770                 | 795               | 796               | 786               |
| 10%                       | 730         | 786                 | 811               | 813               | 807               |
| 20%                       | 768         | 811                 | 834               | 833               | 829               |
| 30%                       | 802         | 830                 | 851               | 853               | 846               |
| 40%                       | 819         | 852                 | 867               | 868               | 859               |
| 50%                       | 847         | 871                 | 880               | 880               | 879               |
| Distillation Residue      |             |                     |                   |                   |                   |
| Per cent of Feed          | 50          | 50.8                | 56.2              | 55.2              | 49.3              |

are properties of the resulting air-blown product and properties after the second stage catalytic treatment.

The data in the foregoing Table are for purposes of illustration only. Such data will vary from time to time in the normal refining of crude oil at any particular refinery. At such times, as one skilled in the art in possession of this disclosure having studied the same will understand, the conditions of the treatment of the feeds will be adjusted to obtain the results desired. Clearly, properties of oils will vary substantially with crude oil source, operating conditions, and the extent to which a particular oil has been fractionated prior to the reactions which are involved in the production of the resin-containing oil of the present invention.

Table II-continued

PREPARATION AND PROPERTIES OF ASPHALTIC RESINS PREPARED FROM  
SYN TOWER BOTTOMS

| Feedstock             | First Stage |      | Second Stage        |        |
|-----------------------|-------------|------|---------------------|--------|
|                       | Air Blowing |      | Catalytic Treatment |        |
| Viscosity, SFS, 210 F | 7.5         | 68.7 | 166.6               | 123.5* |
|                       |             |      |                     | 149.8  |

\*The blend was comprised of about 61 wt % G and 39 wt % of product H.

\*Calculated viscosity from G and J assuming a straight line function.

The preceding data indicate that air blowing of the Syntower bottoms produces a material which, upon distillation, yields a high boiling residue which is considerably more viscous than the corresponding fraction obtained from the untreated syntower bottoms. Further treatment of the airblown product with zinc chloride at about 550 F yields an 880 F+ residue having a much higher viscosity than resulting from air treatment alone. Maximum viscosity increase is obtained when  $ZnCl_2$  is used to treat the air blown intermediate while  $FeCl_3$  and  $SnCl_4$  were each effective to a slightly lesser extent. Neither  $CuCl_2$  nor  $SnCl_4$  were effective in the second stage treatment. These data are reported in Table III.

measuring the viscosity of the distillation residue. Higher viscosities as compared to those of a control containing no catalyst indicate a more reactive catalyst. Based upon viscosity data neither  $CuCl_2 \cdot 2H_2O$  nor  $SnCl_4 \cdot 5H_2O$  were considered effective as second stage catalysts as compared to anhydrous  $ZnCl_2$  or to  $FeCl_3 \cdot 6H_2O$ . Note also that  $ZnCl_2 \cdot 2H_2O$  was not as effective as the anhydrous zinc chloride.

Similar laboratory tests were made to determine the feasibility of using solvent gas oil, produced on the solvent deasphalting unit, as a feedstock for the preparation of asphaltic resins. This feed was considered since the amount of resins which can be prepared from a syn-

Table III

EFFECT OF VARIOUS SECOND-STAGE CATALYSTS  
FOR INCREASING THE VISCOSITY OF THE 880 F+ DISTILLATION RESIDUE DERIVED  
FROM AIR BLOWN SYNTOWER BOTTOMS

| Feedstock                                 | 1st Stage   |         | Second Stage, Catalytic Treatment |                      |          |                      |                      |                      |
|-------------------------------------------|-------------|---------|-----------------------------------|----------------------|----------|----------------------|----------------------|----------------------|
|                                           | Air Blowing | Control | 1                                 | 2                    | 3        | 4                    | 5                    | 6                    |
| Catalyst, Wt %                            | 0           | 0       | 1.0                               | 1.0                  | 1.0      | 1.0                  | 1.0                  | 1.0                  |
| Catalyst                                  | None        | None    | $FeCl_3 \cdot 6H_2O$              | $FeCl_3 \cdot 6H_2O$ | $ZnCl_2$ | $SnCl_4 \cdot 2H_2O$ | $CuCl_2 \cdot 2H_2O$ | $SnCl_4 \cdot 5H_2O$ |
| Composition                               |             |         |                                   |                      |          |                      |                      |                      |
| Reaction                                  |             |         |                                   |                      |          |                      |                      |                      |
| Temp., F                                  | —           | —       | 550                               | 600                  | 540      | 550                  | 550                  | 550                  |
| Reaction Time                             |             |         |                                   |                      |          |                      |                      |                      |
| Hours                                     | —           | —       | 5.75                              | 6.0                  | 6.0      | 6.5                  | 6.0                  | 6.0                  |
| 880 F+ Distillation                       |             |         |                                   |                      |          |                      |                      |                      |
| Residue, Wt %                             | 50          | 50.8    | 50.0                              | 51.2                 | 56.2     | 48.7                 | 53.4                 | 52.8                 |
| Viscosity of 880 F+ Residue, SFS at 210 F | 7.5         | 68.7    | 105.4                             | 108.7                | 166.6    | 82.9                 | 48.0                 | 36.2                 |

Note: In these tests, the initial oil was feedstock A of Table II.

In these tests, syntower bottoms (air blown at 492 F for 3.5 hours in the first stage of the process) were treated at 550 F with 1.0 weight percent catalyst for 5.75 to 6 hours. After this treatment the liquid product was vacuum distilled to yield an 880 F+ bottoms product. Effectiveness of the catalyst was determined by

45 tower bottom alone may not meet the demands for asphalt production. Mixtures of resins derived from the several procedures can be used to produce the final asphalts. Processing details and properties of the airblown intermediate and the  $ZnCl_2$  treated materials are given in Table IV and Table V.

Table IV  
PREPARATION AND PROPERTIES OF ASPHALTIC RESINS PREPARED FROM SOLVENT GAS OILS

|                                             | Feedstock,<br>Solvent<br>Gas Oil | First Stage<br>Air Blowing | Second Stage<br>Catalytic<br>Treatment |
|---------------------------------------------|----------------------------------|----------------------------|----------------------------------------|
| Identification                              | D*                               | —                          | —                                      |
| Catalyst Used                               | —                                | NONE                       | $ZnCl_2$                               |
| Wt. % Catalyst                              | —                                | NONE                       | 1.0                                    |
| Gas Used in Test                            | —                                | $O_2 + steam$              | $CH_4$                                 |
| Gas Rate, SCFH                              | —                                | 2.0                        | < 1                                    |
| Reaction Temperature, °F                    | —                                | 515                        | 560                                    |
| Reaction Time, Hours                        | —                                | 5.5                        | 6.75                                   |
| API Gravity, 60/60° F                       | 23.2                             | —                          | 19.7                                   |
| Specific Gravity, 60/60° F                  | 0.9147                           | —0.9358                    |                                        |
| Distillation, ASTM D 1160                   |                                  |                            |                                        |
| IBP° F                                      | 780                              | —                          | 886                                    |
| 2 %                                         | 805                              | —                          | 923                                    |
| 5 %                                         | 853                              | —                          | 945                                    |
| 10 %                                        | 877                              | —                          | 949                                    |
| 20 %                                        | 913                              | —                          |                                        |
| 30 %                                        | 949                              | —                          |                                        |
| 40 %                                        | 972                              | —                          |                                        |
| 50 %                                        | 985                              | —                          |                                        |
| Distillation Residue<br>Per cent of Product | 61.8                             | 86.8**                     | 88.6                                   |

Table IV-continued

## PREPARATION AND PROPERTIES OF ASPHALTIC RESINS PREPARED FROM SOLVENT GAS OILS

| Feedstock,<br>Solvent<br>Gas Oil | First Stage<br>Air Blowing | Second Stage<br>Catalytic<br>Treatment |
|----------------------------------|----------------------------|----------------------------------------|
| Viscosity, SFS 210° F            | 18.4                       | 27 <sup>(1)</sup>                      |

<sup>(1)</sup>Estimated

\*See Table I

Table V

## PREPARATION AND PROPERTIES OF ASPHALTIC RESINS FROM SOLVENT GAS OIL

| Feedstock<br>Solvent<br>Gas Oil | First Stage,<br>Air Blowing | Second Stage<br>Catalytic<br>Treatment |
|---------------------------------|-----------------------------|----------------------------------------|
| Identification                  | D*                          | —                                      |
| Catalyst Used                   | —                           | —                                      |
| Wt. % Catalyst                  | NONE                        | ZnCl <sub>2</sub>                      |
| Gas Used in Test                | NONE                        | 1.0                                    |
| Gas Rate, SCFH                  | Air                         | CH <sub>4</sub>                        |
| Reaction Temperature, °F        | 2.0                         | <1                                     |
| Reaction Time, Hours            | 550-575                     | 560                                    |
| API Gravity, 60° F              | 7.0                         | 6.0                                    |
| Specific Gravity, 60/60° F      | 23.2                        | 19.4                                   |
| Distillation, ASTM D 1160       | 17.1                        | 17.1                                   |
| IBP °F                          | 0.9147                      | 0.9377                                 |
| 2 %                             | 780                         | 874                                    |
| 5 %                             | 805                         | 901                                    |
| 10 %                            | 853                         | 937                                    |
| 20 %                            | 877                         | 960                                    |
| 30 %                            | 913                         | —                                      |
| 40 %                            | 949                         | —                                      |
| 50 %                            | 972                         | —                                      |
| Distillation Residue            | 985                         | —                                      |
| Per cent of Product             | 61.8                        | 87.6                                   |
| Viscosity, SFS at 210° F        | 18.4                        | 50.5                                   |
|                                 |                             | 94.4                                   |
|                                 |                             | 81.0                                   |

\*Table I

Attention is directed to Table V, showing a substantial increase in viscosity of the distillation residue after the second stage catalytic treatment (81 SFS) as compared to the original feedstock (18.4 SFS) and the air blown intermediate (50.5 SFS). Higher viscosity (81.0 SFS) of the distillation residue is obtained upon ZnCl<sub>2</sub> catalytic treatment when the gas oil is subjected to more severe air blowing (Table V) prior to the second stage catalytic treatment as compared to the less severe air blowing of Table IV (viscosity of 35.9 SFS).

The material obtained as the distillation residue after the two-stage treatment in Table V having a viscosity of 81 SFS was very tacky and resembled the resins separated from paving asphalts by other methods.

Additional tests have been made to determine whether a combination of syntower bottoms and solvent gas oil could be used as a feedstock for the production of synthetic resins. While the reaction mechanism is not known, it is believed that the more aromatic components of the feedstocks are possibly alkylated in the presence of ZnCl<sub>2</sub> with the more paraffinic materials. Therefore, a mixture of air blown syntower bottoms, which are more aromatic, and air blown solvent gas oil which is paraffinic, should result in a highly resinous material with properties substantially different from those of corresponding products obtained from each of the separate feedstocks. Preparation and some properties of the resins from the mixed air blown feedstocks are shown in Table VI.

Table VI

| Charge                     | Feedstock           |                    | First Stage<br>Air Blowing |                    | Second Stage<br>Catalytic |
|----------------------------|---------------------|--------------------|----------------------------|--------------------|---------------------------|
|                            | Syntower<br>Bottoms | Solvent<br>Gas Oil | Syntower<br>Bottoms        | Solvent<br>Gas Oil |                           |
| Identification             | B <sup>(1)</sup>    | D <sup>(1)</sup>   | —                          | —                  | Blend*                    |
| Catalyst Used              | NONE                | NONE               | NONE                       | NONE               | ZnCl <sub>2</sub>         |
| Wt. % Catalyst             | NONE                | NONE               | NONE                       | NONE               | 1                         |
| Gas Used                   | —                   | —                  | Air                        | Air                | CH <sub>4</sub>           |
| Gas Rate, SCFH             | —                   | —                  | 2.0                        | 2.0                | 1.0                       |
| Reaction Temperature, °F   | —                   | —                  | 375                        | 530                | 560                       |
| Reaction Time, Hours       | —                   | —                  | 2.5                        | 6.0                | 5.5                       |
| API Gravity, 60° F         | 13.6                | 23.2               | —                          | —                  | 13.7                      |
| Specific Gravity, 60/60° F | 0.9752              | 0.9147             | —                          | —                  | 0.9745                    |
| Distillation, ASTM D 1160  |                     |                    |                            |                    |                           |
| IBP °F                     | 564                 | 780                | —                          | —                  | 693                       |
| 2 %                        | 571                 | 805                | —                          | —                  | 743                       |
| 5 %                        | 680                 | 853                | —                          | —                  | 780                       |
| 10 %                       | 730                 | 877                | —                          | —                  | 817                       |
| 20 %                       | 768                 | 913                | —                          | —                  | 853                       |
| 30 %                       | 802                 | 949                | —                          | —                  | 889                       |
| 40 %                       | 819                 | 972                | —                          | —                  | 935                       |
| 50 %                       | 847                 | 985                | —                          | —                  | —                         |
| Distillation Residue       |                     |                    |                            |                    |                           |
| Per cent of Product        | 50                  | 61.8               | —                          | —                  | 56.0                      |

Table VI-continued

| Charge                   | Feedstock           |                    | First Stage         |                    | Second Stage |
|--------------------------|---------------------|--------------------|---------------------|--------------------|--------------|
|                          | Syntower<br>Bottoms | Solvent<br>Gas Oil | Syntower<br>Bottoms | Solvent<br>Gas Oil |              |
| Viscosity, SFS at 210° F | 7.5                 | 18.4               | —                   | —                  | 72.2         |

\*Blend consisted of 47.4 wt. % air blown syntower bottoms and 52.3 wt. % blown solvent gas oil.

\*\*Table I

While the actual viscosity of the distillation residue of the blend of air blown syntower bottoms and air blown solvent gas oil followed by second stage catalytic treatment was 72.2 SFS at 210° F., the material was tacky and resembled resins separated from paving asphalts by various methods.

These results confirm that resinous materials are formed by the preceding sequence of reactions. However, the viscosity increase in this example is believed to be minimum and is expected to increase with an increase in the severity of the air blowing at higher temperatures of the syntower bottoms. Feedstocks that can be used in this invention are those containing a substantial amount of aromatics, i.e., at least about 15 percent aromatics to obtain ordinarily economically feasible results. That is, sufficient aromatics must be available to form reasonable quantities of resin in the oil subjected to the two-stage treatment of the invention; syntower bottoms, light and heavy cycle oils, phenol extract oils,  $\text{SO}_2$  extract oil, vacuum and solvent extract oils.

Properties of feedstocks which are suitable for the preparation of synthetic resins for use as asphalt additives are given in Table VII.

Table VII

PROPERTIES OF FEEDSTOCKS  
SUITABLE FOR THE PREPARATION OF SYNTHETIC RESINS  
FOR USE AS ASPHALT ADDITIVES

|                                     | Range of Properties |           | 45 |
|-------------------------------------|---------------------|-----------|----|
|                                     | Broad               | Preferred |    |
| API Gravity, 60° F                  | 2.0-30.             | 5.0-25.0  |    |
| Aniline Point, °F                   | 75-230              | 85-185    |    |
| Viscosity, SFS, 122° F              | 5-500               | 25-250    |    |
| H/C Mol Ratio                       | 1.2-2.0             | 1.3-1.8   |    |
| IBP, °F                             | 500-1000            | 575-800   |    |
| 50%, Point, °F                      | 700-1100            | 800-1000  |    |
| Carbon Residue, Rams., %            | 0.2-18.             | 0.5-15.   |    |
| No. Avg. Mol. Wt.                   | 200-1000            | 300-600   |    |
| Paraffin Hydrocarbon Content, Wt. % | 0.1-80              | 10-50     |    |

The temperature for air blowing may range from about 350° to about 600° F., preferably 400° to 550° F.

The temperature of the catalytic treatment may range from about 500° F to about 600° F, preferably 530° to 570° F.

The selected temperature, in any case, whether within or outside the given ranges can be determined by test.

When compared with corresponding asphaltic materials obtained from the same feedstock containing none of the added synthetic resins, asphalts prepared in the manner disclosed in this invention have improved quality as determined by viscosity, ductility and other temperature dependent characteristics.

15 While the asphalt prepared in accordance with this invention can be prepared in a number of different ways, the following method illustrates the process and shows the improvement in the properties of the final asphaltic product containing the synthetic resins.

20 Ordinarily, the amount of resin-containing oil from the second stage or catalytic treatment added to a topped crude or to an asphalt will be in the range of from about 1/10 to about 10 weight percent, or more, depending upon the properties of the resin, and, of course, of the final asphalt desired to be obtained.

25 It is possible within the scope of the appended claims to first treat the second stage catalytically treated, resin-containing oil to remove the oil therefrom, as by solvent deoiling, and to recover resin and to then add the thus concentrated resin to an asphalt cement to improve its properties. In such instance, the proportion of resin added can be smaller understandably because with oil has been largely, if not completely, removed from the resin.

30 The a priori treatment to concentrate the resin is not now preferred because this involves additional steps and equipment. Obviously, the addition of the resin containing oil to a topped crude, which is to be a vacuum distilled and/or solvent deasphalted, is more attractive from an economic viewpoint.

35 In the following Table VIII product J of Table II, obtained by the successive dual stage treatment of "syntower" bottoms with air and then with  $\text{ZnCl}_2$  at temperatures ranging from 250 to about 600 F, was added to a 430 F+ topped crude representing the current total charge to the refinery. The mixture thus obtained contained 4 wt. percent of the synthetic resin fraction. It was further distilled to yield a 650 F+ bottoms which was subsequently charged to a semi-continuous isothermal vacuum flash distillation unit to yield various grades of asphalt cements for use in highway paving applications. These asphalts containing the synthetic resins are compared to similar materials, in the following tabulations, derived from the same 430 F+ topped crude but which contained no additive. Solvent extraction can be employed with even greater success, to yield asphalts of improved quality from the 650 F+ topped crude.

40 According to the invention, the synthetic resins can be concentrated by either vacuum reduction or by solvent extraction and then added to asphalt previously produced by some other means. It is within the scope of the invention to at least partly effect a concentration of the resins containing product, to then admix it with a topped crude or asphalt and to then produce the final asphaltic product as herein described. In either instance more resinous portion of the reaction product would remain in the final asphaltic residue.

Table VIII

EFFECT OF SYNTHETIC RESINS DERIVED FROM SYNTOWER BOTTOMS  
ON THE PROPERTIES OF TOPPED CRUDES AND ASPHALTS  
FROM SIMULATED CRUDES CHARGED TO THE  
REFINERY

| Composition of Feed                 | Control | Additive Blend |       |       |         |
|-------------------------------------|---------|----------------|-------|-------|---------|
| Topped Crude, 430 F+, wt %          | 100.0   | 96.0           |       |       |         |
| Product J*, wt %                    | 0.0     | 4.0            |       |       |         |
| API Gravity, 60 F                   | 26.1    | 25.3           |       |       |         |
| Distn. to Yield 650 F+ Btms.        |         |                |       |       |         |
| Yield, vol % of 450 F+ Feed         | 59.0    | 59.4           |       |       |         |
| API Gravity at 60 F                 | 20.3    | 19.0           |       |       |         |
| Specific Gravity, 60/60 F           | 0.9321  | 0.9402         |       |       |         |
| Viscosity, SUS at 210 F             | 112.0   | 114.1          |       |       |         |
| Viscosity, SFS at 122 F             | 93.2    | 134.7          |       |       |         |
| Pour Point, F                       | +95     | +100           |       |       |         |
| Sulfur, Wt %                        | 1.60    | 1.46           |       |       |         |
| Carbon Residue, Rams., %            | 0.02    | 0.02           |       |       |         |
| Ash, Wt. %                          | 0.02    | 0.02           |       |       |         |
| Ni, ppm                             |         | 14.7           |       |       |         |
| Fe, ppm                             |         |                |       |       |         |
| V, ppm                              |         | 22.2           |       |       |         |
| Vacuum Asphalt Properties           | Control | Additive Blend |       |       |         |
| Test No.                            | 1       | 2              | 3     | 4     | 5       |
| Cor. Flash Temp., F                 | 960     | 975            | 955   | 960   | 975     |
| Yield, vol % of 430 F+              | 36.4    | 33.6           | 36.6  | 35.6  | 36.4    |
| API Gravity at 60 F                 | 9.9     | 9.1            | 9.0   | 9.1   | 8.4     |
| Penetration, mm/10                  |         |                |       |       |         |
| 200 g/60 sec/39.2 F                 | 35      | 25             | 33    | 29    | 24      |
| 100 g/5 sec/77 F                    | 135     | 73             | 129   | 113   | 66      |
| Penetration Ratio                   | 25.9    | 34.2           | 25.6  | 25.7  | 36.4    |
| Viscosity                           |         |                |       |       |         |
| SFS, 210 F                          | 442     | 849            | 524   | 580   | 981     |
| SFS, 275 F                          | 70.7    | 112.4          | 79.4  | 85.3  | 125.0   |
| Poises, 140 F                       | 265.3   | 862.4          | 332.1 | 478.0 | 1,067.1 |
| Ductility, cm                       |         |                |       |       |         |
| 1 cm/min., 39.2 F                   | 4.5     | 6.5            | 5.5   | 4.5   | 4.0     |
| 5 cm/min., 77 F                     | 86      | 108            | 115   | 113   | 150+    |
| Softening Point, R & B, F           | 118     | 124            | 115   | 118   | 123     |
| Spot Test (1)                       | Pos     | Pos            | Pos   | Pos   | Pos     |
| Solubility, CCl <sub>4</sub> , wt % | 99.94   | 99.83          | 99.53 | 99.85 | 99.97   |

(1) Positive spot denotes the presence of wax, not cracking.

\*Table II

Table IX

PREPARATION AND PROPERTIES OF ASPHALTIC RESINS PREPARED FROM  
SOLVENT GAS OIL FEEDSTOCK D (TABLE I)

|                            | First Stage         |        | Second Stage        |                   |                   |
|----------------------------|---------------------|--------|---------------------|-------------------|-------------------|
|                            | Air Blowing         |        | Catalytic Treatment |                   | P<br>Blend*       |
| Run Number                 | K                   | L      | M                   | N                 |                   |
| Material Charged           | D                   | K      | L                   | K                 |                   |
| Catalyst used              | NONE                | NONE   | ZnCl <sub>2</sub>   | ZnCl <sub>2</sub> |                   |
| Wt. % Catalyst             | NONE                | NONE   | 1.0                 | 1.0               |                   |
| Gas used in test           | air                 | air    | CH <sub>4</sub>     | CH <sub>4</sub>   |                   |
| Gas rate, SCFH             | 2.0                 | 2.0    | <1                  | <1                |                   |
| Reaction Temperature, °F.  | 515                 | 550    | 560                 | 560               |                   |
| Reaction Time, Hours       | 5.5                 | 7.0    | 6.0                 | 6.75              |                   |
| API Gravity at 60° F.      | —                   | 19.4   | 17.1                | 19.7              | 18.1              |
| Specific Gravity, 60/60°F. | —                   | 0.9377 | 0.9522              | 0.9358            | 0.9459            |
| ASTM D 1160 Distillation   |                     |        |                     |                   |                   |
| IBP °F.                    | —                   | 874    | 901                 | 886               |                   |
| 2%                         | —901                | 945    | 923                 |                   |                   |
| 5%                         | —                   | 937    | 972                 | 945               |                   |
| 10%                        | —                   | 960    | —                   | 949               |                   |
| Distillation Residue       |                     |        |                     |                   |                   |
| Percent of Product         | 88.8 <sup>(2)</sup> | 87.6   | 94.4                | 88.6              |                   |
| Viscosity, SFS, 210° F.    | 27 <sup>(3)</sup>   | 50.5   | 81.0                | 35.9              | 63 <sup>(4)</sup> |

\*Blend of 40 wt. % of Run N and 60 wt. % of Run M.

<sup>(1)</sup>Calculated viscosity from Run N & M assuming a straight line function.<sup>(2)</sup>Estimate.

Similar tests were made in which synthetic resins prepared from solvent gas oil, Table IX, was used as an additive for the 430 F+ topped which was then topped to

650 F and vacuum flashed to yield asphalts. Results follow in Table X:

Table X

EFFECT OF SYNTHETIC RESINS DERIVED FROM SOLVENT GAS OIL  
ON THE PROPERTIES OF TOPPED CRUDES AND ASPHALTS  
FROM SIMULATED CRUDES CHARGED TO THE  
REFINERY

| Composition of Feed                 | Control | Additive Blend |       |       |
|-------------------------------------|---------|----------------|-------|-------|
| Topped Crude, 430 F+, wt %          | 100.0   | 96.0           |       |       |
| Product P*, wt %                    | 0.0     | 4.0            |       |       |
| API Gravity, 60 F                   | 26.1    | 25.8           |       |       |
| <u>Distn. to Yield 650 F+ Btms.</u> |         |                |       |       |
| Yield, vol % of 450 F+ Feed         | 59.0    | 59.9           |       |       |
| API Gravity at 60 F                 | 20.3    | 20.1           |       |       |
| Specific Gravity, 60/60 F           | 0.9321  | 0.9334         |       |       |
| Viscosity, SUS at 210 F             | 112.0   | 124.1          |       |       |
| Viscosity, SFS at 122 F             | 93.2    | 128.4          |       |       |
| Pour Point, F                       | +95     | +100           |       |       |
| Sulfur, wt %                        | 1.60    | 1.40           |       |       |
| Carbon Residue, Rams., %            | 6.73    | 7.59           |       |       |
| Ash, wt %                           | 0.02    | 0.04           |       |       |
| Ni, ppm                             |         |                |       |       |
| Fe, ppm                             |         |                |       |       |
| V, ppm                              |         | 12.0           |       |       |
| <u>Vacuum Asphalt Properties</u>    |         |                |       |       |
|                                     | Control | Additive Blend |       |       |
| Test No.                            | 1       | 2              | 6     | 7     |
| Cor. Flash Temp., F                 | 960     | 975            | 960   | 970   |
| Yield, vol % of 430 F+              | 36.4    | 33.6           | 39.7  | 38.8  |
| API Gravity at 60 F                 | 9.9     | 9.1            | 10.4  | 10.3  |
| <u>Penetration, mm/10</u>           |         |                |       |       |
| 200 g/60 sec/39.2 F                 | 35      | 25             | 46    | 37    |
| 100 g/5 sec/77 F                    | 135     | 73             | 185   | 146   |
| Penetration Ratio                   | 25.9    | 34.2           | 24.9  | 25.3  |
| <u>Viscosity</u>                    |         |                |       |       |
| SFS, 210 F                          | 442     | 849            | 319   | 441   |
| SFS, 275 F                          | 70.7    | 112.4          | 58.2  | 71.1  |
| Poises, 140 F                       | 265.3   | 862.4          | 171   | 291.6 |
| <u>Ductility, cm</u>                |         |                |       |       |
| 1 cm/min., 39.2 F                   | 4.5     | 6.5            | 11.5  | 6.5   |
| 5 cm/min., 77 F                     | 86      | 108            | 54    | 59    |
| Softening Point, R&B, F             | 118     | 124            | 115   | 118   |
| Spot Test (1)                       | Pos     | Pos            | Pos   | Pos   |
| Solubility, CCl <sub>4</sub> , wt % | 99.94   | 99.83          | 99.90 | 99.95 |
| 99.90                               | 99.95   | 99.90          | 99.95 |       |

(1) Positive spot denotes the presence of wax, not cracking.

\*See Table IX

The preceding test data show that synthetic asphaltic resins prepared by the two-stage treatment of syntower 45 and solvent gas oil were effective as additives for improving the quality of paving asphalts derived from crudes being processed at a refinery.

The second tabulation shows that similar resins prepared from the solvent gas oil derived from the same crudes in the plant were not as effective. Since solvent extraction would have been used to prepare the asphalts in the plant instead of vacuum reduction, which was used in the laboratory, more of the unreacted paraffinic portions of the solvent gas oil additive would have been extracted from the asphalt, thereby leaving more aromatic resins in the asphalt phase. Therefore it is contended, reasonably and as one skilled in the art will understand, that further improvement in the ductility of asphalts prepared by solvent extraction to the 650 F+ feed would have been apparent than observed for the vacuum asphalts prepared in the laboratory.

A similar series of tests were made in which a mixture of air blown and ZnCl<sub>2</sub> treated syntower bottoms and solvent gas oil was added to the 430 F+ topped crude which was then further distilled and vacuum flashed to yield asphalts. Results are presented in Tables XI and XII.

Table XI  
PREPARATION AND PROPERTIES OF RESINS PREPARED  
FROM A  
MIXTURE OF SYNTOWER BOTTOMS AND SOLVENT GAS OIL

| 50                          | Product No.               | First Stage      |                 | Second Stage        |
|-----------------------------|---------------------------|------------------|-----------------|---------------------|
|                             |                           | Syntower Bottoms | Solvent Gas Oil | Catalytic Treatment |
| 55                          | Charge to Run             | A                | D               | R                   |
|                             | Identification**          | NONE             | NONE            | ZnCl <sub>2</sub>   |
|                             | Catalyst Used             | NONE             | NONE            | 1%                  |
|                             | Wt. % Catalyst            | air              | air             | CH <sub>4</sub>     |
|                             | Gas Used                  | 2.0              | 2.0             | 1.0                 |
|                             | Gas Rate, SCFH            | 375              | 530             | 560                 |
|                             | Reaction Temperature, °F  | 2.5              | 6.0             | 5.5                 |
|                             | Reaction Time, Hours      | —                | —               | 13.7                |
|                             | API Gravity, 60°F         | —                | —               | 0.9745              |
| 60                          | Specific Gravity, 60/60°F | —                | —               |                     |
| <u>ASTM D 1160 Distn.</u>   |                           |                  |                 |                     |
|                             | IBP °F                    | —                | —               | 693                 |
|                             | 2%                        | —                | —               | 743                 |
|                             | 5%                        | —                | —               | 780                 |
|                             | 10%                       | —                | —               | 817                 |
|                             | 20%                       | —                | —               | 853                 |
|                             | 30%                       | —                | —               | 889                 |
|                             | 40%                       | —                | —               | 935                 |
| <u>Distillation Residue</u> |                           |                  |                 |                     |
|                             | Percent of Product        |                  |                 | 56.0                |

Table XI-continued

PREPARATION AND PROPERTIES OF RESINS PREPARED  
FROM A  
MIXTURE OF SYNTOWER BOTTOMS AND SOLVENT GAS OIL

|                       | First Stage<br>Air Blowing | Second<br>Stage<br>Catalytic<br>Treatment | 5  |
|-----------------------|----------------------------|-------------------------------------------|----|
| Viscosity, SFS, 210°F |                            | 72.2                                      | 10 |

\*Blend consisted of 47.7 wt. % A and 52.3 wt. % D.

\*\*See Table I

process comprises (1) air blowing a hydrocarbon oil fraction having the following properties:

API Gravity, 60°F, 2.0-30  
 Aniline Point, °F, 75-230  
 Viscosity, SFS, 122°F, 5-500  
 H/C Mol Ratio, 1.2-2.0  
 IBP, °F, 500-1000  
 50 percent Point, °F, 700-1000  
 Carbon Residue, Rams., percent, 0.2-18  
 No. Avg. Mol. Wt., 200-1,000  
 Paraffin Hydrocarbon Content, Wt. percent, 0.1-80  
 at an elevated temperature in the range of from about

Table XII

EFFECT OF SYNTHETIC RESINS DERIVED FROM SYNTOWER BTMS. AND SGO  
ON THE PROPERTIES OF TOPPED CRUDES AND ASPHALTS  
FROM SIMULATED CRUDES CHARGED TO THE  
REFINERY

| Composition of Feed                  | Control        | Additive Blend        |       |       |
|--------------------------------------|----------------|-----------------------|-------|-------|
| Topped Crude, 430 F+wt %             | 100.0          | 96.0                  |       |       |
| Product R*, wt. %                    | 0.0            | 4.0                   |       |       |
| API Gravity, 60 F                    | 26.1           | 25.8                  |       |       |
| <u>Distn. to Yield 650 F+ Btms.</u>  |                |                       |       |       |
| Yield, vol % of 450 F+ Feed          | 59.0           | 59.1                  |       |       |
| API Gravity at 60 F                  | 20.3           | 19.6                  |       |       |
| Specific Gravity, 60/60 F            | 0.9321         | 0.9365                |       |       |
| Viscosity, SUS at 210 F              | 112.0          | 118.6                 |       |       |
| Viscosity, SFS at 122 F              | 93.2           | 95.7                  |       |       |
| Pour Point, F                        | +95            | +100                  |       |       |
| Sulfur, wt. %                        | 1.60           | 1.45                  |       |       |
| Carbon Residue, Rams., %             | 6.73           | 7.03                  |       |       |
| Ash, wt. %                           | 0.02           | 0.03                  |       |       |
| <u>Vacuum Asphalt Properties</u>     | <u>Control</u> | <u>Additive Blend</u> |       |       |
| Test No.                             | 1              | 2                     | 9     | 10    |
| Cor. Flash Temp., F                  | 960            | 975                   | 960   | 965   |
| Yield, vol % of 430 F+               | 36.4           | 33.6                  | 37.8  | 34.9  |
| API Gravity at 60 F                  | 9.9            | 9.1                   | 10.0  | 9.5   |
| <u>Penetration, mm/10</u>            |                |                       |       |       |
| 200 g/60 sec/39.2 F                  | 35             | 25                    | 38    | 34    |
| 100 g/ 5 sec/77 F                    | 135            | 73                    | 160   | 133   |
| Penetration Ratio                    | 25.9           | 34.2                  | 23.8  | 25.6  |
| <u>Viscosity</u>                     |                |                       |       |       |
| SFS, 210 F                           | 442            | 849                   | 373   | 470   |
| SFS, 275 F                           | 70.7           | 112.4                 | 62.2  | 72.4  |
| Poises, 140 F                        | 265.3          | 862.4                 | 187.9 | 261.0 |
| <u>Ductility, cm</u>                 |                |                       |       |       |
| 1 cm/min., 39.2 F                    | 4.5            | 6.5                   | 10.5  | 7.0   |
| 5 cm/min., 77 F                      | 86             | 108                   | 76    | 76    |
| Softening Point, R&B, F              | 118            | 124                   | 113   | 116   |
| Spot Test (1)                        | Pos            | Pos                   | Pos   | Pos   |
| Solubility, CCl <sub>4</sub> , wt. % | 99.94          | 99.83                 | 99.96 | 99.93 |
|                                      |                |                       |       | 99.98 |

(1) Positive spot denotes the presence of wax, not cracking.

\*Table XI

Reasonable modification are possible within the scope of the foregoing disclosure and the appended claims to the invention the essence of which is that there are produced by a combination of steps, i.e., air blowing at elevated temperature and then while still at elevated temperature treating with a catalyst an oil as herein described to produce a petroleum resin containing material which then, according to the invention, as such or in at least partly concentrated form is added to a topped crude or asphalt or similar material from which a final asphalt of, say, paving grade can be produced as by vacuum distillation, solvent extraction or otherwise as may be desired.

We claim:

1. A process for producing an additive, suitable for use in the production of high quality asphalt usable for paving said additive containing petroleum resin, which

55 350° to about 600°F for a period of time sufficient at said temperature to produce a treated fraction containing resin-forming materials and (2) subsequently, heating to a temperature in the range of about 500° to about 600°F said treated fraction in the presence of a catalyst chosen from among ZnCl<sub>2</sub>, FeCl<sub>3</sub>, and SnCl<sub>2</sub> to produce a treated hydrocarbon oil fraction which contains petroleum resin.

2. A process for the preparation of an asphalt suitable for producing paving grade asphaltic material which 60 comprises incorporating a petroleum resin-containing material of claim 1 into a base material selected from among an asphalt and topped crude to produce a mixture and removing hydrocarbon oil from said mixture to recover an asphalt containing said petroleum resin.

3. A process according to claim 1 wherein the petroleum resin-containing materials are derived from a first bottoms fraction derived in fractionating a synthetic

hydrocarbon mixture produced in a catalytic cracking of virgin gas oil.

4. An operation according to claim 2 wherein the petroleum resin-containing material is first treated to remove hydrocarbon oil at least partly thereby concentrating said petroleum resin-containing material and then said petroleum resin-containing material is added to said base material.

5. A method of improving an asphalt which comprises recovering the resin from the product of claim 1 and adding the recovered resin to an asphalt.

6. A method according to claim 5 wherein the product of claim 1 is solvent deoiled to obtain concentrated resin and said concentrated resin is added to the asphalt.

7. Operation of claim 2 wherein said removing of hydrocarbon oil is by vacuum distillation.

8. The method of claim 2 wherein said removing of hydrocarbon oil is by solvent extraction.

9. The method of claim 4 wherein said removing of hydrocarbon oil is by vacuum distillation.

10. The method of claim 4 wherein said removing of hydrocarbon oil is by solvent extraction.

\* \* \* \* \*